

# UNITED STATES PATENT OFFICE.

WILLIAM N. BLAKEMAN, JR., OF MOUNT VERNON, NEW YORK.

## PROCESS OF IMPARTING DRYING PROPERTIES TO OILS.

SPECIFICATION forming part of Letters Patent No. 496,991, dated May 9, 1893.

Application filed January 31, 1893. Serial No. 460,190. (No specimens.)

*To all whom it may concern:*

Be it known that I, WILLIAM N. BLAKEMAN, Jr., of Mount Vernon, in the county of Westchester and State of New York, have invented 5 a new and useful Process of Imparting Drying Properties to Oils, as well as hastening drying action, where it exists in the same, which invention is fully set forth in the following specification.

10 The object of this invention is to impart drying properties to those oils, either animal or vegetable, which belong to the so called, fatty, or "non-drying"--class, as well as to hasten the drying action of those oils which 15 are technically denominated "drying oils."

The invention will first be particularly described and then set forth in general in the claims.

Animal and vegetable oils are known as 20 oxygenated hydrocarbons, that is they are composed of oxygen, hydrogen and carbon, and have the natural characteristic of taking on more oxygen by absorption when exposed to the air, the "drying oils" in such case becoming resinous, and the non-drying oils becoming thick and viscous. It is also known 25 that this acidifying element of oxygen can be further increased artificially by exposure of the oils to a continuous current or atmosphere 30 of oxygen, or by heating or "boiling on oxygen-carriers," such as the metallic oxides, and oxy-salts, or by adding to them, in their cold state, some of said oxides or salts, as acidifying agents, notably in the form of commercial 35 "paint driers." But although oxygen is the great acidifying agent, it is not alone in this action, chlorine and other elements being classed, as such agents; and oxygen in its union with oils gives acid reactions with the 40 evolution of carbonic acid. In my process I take advantage of this known characteristic, and, therefore, I first, cause the oils to absorb oxygen by admixture with an oxidizing or acidifying agent, and secondly, I cause 45 them to absorb carbonic acid.

The boiling of the oils can be carried on by applying heat directly to the containing vessel, or through the medium of the sand bath, or water bath, and the proportion of oxides 50 used may be from three to five per cent., the boiling requiring two to five hours, the time varying according to the gravity of the oil,

and the oxygen carrier used. But as the boiling points of oils vary between from about 590° to about 620° Fahrenheit, and as these 55 points of temperature are also very near the decomposing points of the oils, care must be exercised that the body and quality of the oils are not injured in the boiling. This danger of injury can be avoided, however, by the 60 use of a steam jacket or water bath, which, while maintaining a much lower temperature, requires a longer exposure to its heat. The agents generally used for the above purposes, are the oxides and salts of lead, such as 65 litharge, minium, and the acetates of lead, also oxides and salts of manganese. After cooling and settling, the oil is ready for the second step of my process, that of imparting to it carbonic acid. This I accomplish by dissolving, grinding or mixing with the oil and by the aid of heat, if necessary, any agent 70 that will absorb carbonic acid from the air, or that will give up carbonic acid having held it in combination, and thus impart it to 75 the oil. I prefer to use for this purpose, those agents which have an affinity for, and will absorb carbonic acid, such as some of the metallic soaps, as alumina, magnesia, or alum soap, and monometaborate of soda, sulphate 80 of magnesia, sulphate of alumina, borate of magnesia, basic acetate of lead, alum and the like chemical agents. One or more of these agents may be used, as the result desired and practice shall dictate, but the best effects are 85 obtained by using those agents which have the property of making the oil alkaline or basic in addition to their power for absorbing carbonic acid, or which have an affinity 90 for the oil and also for carbonic acid, such as magnesia, or alumina soap, and basic acetate of lead, and any of the others may be afterward added such as borate of magnesia, and mono-metaborate of soda. The quantity 95 of these agents used must be governed also largely by practice, but about five per cent. of metallic soap, ten per cent. of borate of magnesia, and fifteen per cent. of basic acetate of lead will give good results. After this treatment carbonic acid may be charged 100 through the oil, and any of the commercial oil driers added without departing from my invention.

A possible explanation of the apparent

paradox, which I effect, that of an acidifying agent giving an acid reaction, and carbonic acid being evolved, and an alkaline or basic agent giving an alkaline or basic reaction and carbonic acid being absorbed, said actions going on apparently interchangeably, seems to be, that the acidifying agent unites progressively with a portion of the oil, evolving and setting free carbonic acid which is 5  
10 immediately seized and absorbed by a portion of the oil rendered alkaline or basic, and this action and reaction continue until mutual exhaustion or until a neutral point is reached.

Having thus fully described my invention, 15 I claim—

1. The process of imparting drying properties to oils, or hastening the drying action of the same, consisting in first chemically combining with the oil an acidifying agent and 20 then adding a carbonating agent, substantially as set forth.

2. The hereinbefore described process of causing oils to absorb carbonic acid, which consists in chemically combining with the 25 oil an acidifying agent and then adding a basic agent capable of absorbing carbonic

acid, substantially as and for the purposes set forth.

3. The hereinbefore described process of causing oils to absorb carbonic acid, which 30 consists in chemically combining with the oil an acidifying agent and then adding an alkaline agent capable of absorbing carbon-dioxide, substantially as and for the purposes set forth.

35 4. The process of imparting drying properties to oils, or hastening the drying action of the same, consisting in first oxidizing, by boiling the oil in mixture with an "oxygen carrier," and then adding a basic agent capable 40 of absorbing carbonic acid, substantially as set forth.

5. The process of imparting drying properties to oils, or hastening the drying action of the same, consisting in first oxidizing, by 45 boiling the oil mixture with an "oxygen carrier," and then adding an alkaline agent, substantially as set forth.

WM. N. BLAKEMAN, JR.

Witnesses:

FRANCIS P. REILLY,  
THEO. H. FRIEND.